# EUROPEAN PATENT SPECIFICATION

(11) **EP 0 074 446 B1**
(45) Date of publication and mention of the grant of the patent: **22.05.1985**
(21) Application number: 81304214.0
(22) Date of filing: 15.09.1981
(51) Int. Cl.: D01D 5/30, D01D 5/24

(54) **Multifilament yarn and spinning process therefor**
Multifilamentgarn und Spinnverfahren
Fil multifilament et procédé de filage

(43) Date of publication of application: 23.03.1983
(73) Proprietor: MONSANTO COMPANY, St. Louis, Missouri 63167 (US)
(72) Inventor: Yu, Jing-peir, Pensacola Florida 32504 (US)
(74) Representative: McLean, Peter

## Description

The invention relates to the art of spinning conjugate filaments splittable into sub-filaments having different deniers. More particularly, it relates to control of the properties of the sub-filaments.

A more natural hand in fabrics made from melt spun yarns is attained when the yarns are composed of filaments having different deniers. A simple known method of making yarns of mixed dpf (denier per filament) is to spin a polymer through a spinneret having capillaries of various lengths and/or cross-sectional areas. To spin a yarn from such a spinneret presents processing difficulties because of the effect of transverse quenching air on the resulting molten streams having different surface areas presented to the quenching air. Large molten streams will be blown further away from the quench air source than small ones. One must accordingly design and install the spinneret such that the small streams are nearest the quench air source, to avoid having the large streams be blown into the small streams. Furthermore, in such a process the quenching rates and the stresses on the large and small streams are different, causing morphological differences in the resulting filaments. Such differences cause variable dyeability and other problems.

According to the invention, these and other difficulties are avoided as will be set forth below. According to a first aspect of the invention, there is provided a spinning process, comprising generating a plurality of molten streams from a spinneret, the streams being formed from axially extending continuous segments of dissimilar polymers arranged alternately in side-by-side temporarily adhering relationship; quenching the streams to form filaments; and withdrawing the filaments from the streams, the streams being selected such that first and second of the filaments have substantially the same denier and are splittable into different numbers of sub-filaments derived from said segments.

According to another aspect of the invention, the streams from which the first and the second of the filaments are quenched have substantially the same jet stretch.

According to another aspect of the invention, there is provided a multi-filament yarn comprising a plurality of filaments of equal deniers splittable into sub-filaments of at least first and second polymers, at least one of the sub-filaments of the first polymer split from a first of the filaments having a different denier than another of the sub-filaments of the first polymer split from a second of the filaments.

According to another aspect of the invention, the first and the second of the filaments are splittable into different numbers of sub-filaments.

Other aspects will in part appear hereinafter and will in part be obvious from the following detailed description taken in connection with the accompanying drawing, wherein:
Figure 1 is a bottom plan view of a spinneret for making yarns according to the invention; and
Figure 2 is a fragmentary perspective view of an exemplary filament according to the invention.

As shown in Figure 1, the preferred spinneret construction illustrated includes several groups of generally arched or horseshoe-shaped slots 20 in spinneret blank 22, those slots 20 in each group being arranged symmetrically about a central point for that group with the open end of the horseshoe shapes facing inwardly. The several slots 20 in each group constitute a combined orifice for spinning a single filament. Slots 20 extend entirely through blank 22 except for recessed web 24 at the apex of each slot 20, the webs 24 and the lands between adjacent ends of slots 20 providing support to retain the material in the center of the combined orifice.

The two dissimilar polymers are fed to combined orifices as sheath-core supply streams, with dotted circles 26 representing the interfaces between the two polymers. Adjacent ends of adjacent slots 20 are sufficiently close that the streams issuing therefrom unite just below the spinneret. The molten spun streams are thus hollow structures composed of alternating axially extending segments of the two polymers. Surface tension and other effects tend to make the molten streams approach hollow circular cross-sections prior to solidification, as shown in Figure 2, which illustrates a filament formed by a combined orifice composed of eight slots 20. If the polymers differ in melt viscosity, it is ordinarily preferable to provide the polymer having the lower viscosity as the core of the stream approaching each combined orifice.

The various slot dimensions in the directions parallel to and transverse to the direction of polymer flow are selected to control the relative deniers of the combined filaments spun from the various combined orifices. Most conveniently, the various slots may be identical in their transverse dimensions, with their lengths parallel to the direction of polymer flow selected to control the relative combined filament deniers. Thus, the three slots 20 for the combined orifice in the upper right corner of Figure 1 may be made shorter in the direction parallel to polymer flow than the six slots 20 for the combined orifice in the lower left corner of Figure 1, so that the combined filaments spun therefrom have substantially the same denier. The molten streams will thus have substantially the same quenching rate and be subjected to substantially the same stresses during spinning, so that the resulting sub-filaments of the same polymer type will dye substantially the same although they may be of substantially different deniers.

Exemplary dissimilar polymers are poly-(ethylene terephthalate) and nylon 66. By "dissimilar" is meant that the polymeric components in the solidified filaments can be readily separated from one another into sub-filaments.

The hand of fabrics made from yarns according to the invention can be varied widely by selection of substantially different deniers for the sub-filaments. Marked improvement in hand occurs when some sub-filaments have deniers at least 50% larger than others of the sub-filaments, with better results when the difference is at least 100%.

Yarns according to the invention can be produced by spinning followed by drawing, either in a coupled process or as separate operations, or can be produced by spinning at speeds sufficiently high as to eliminate the need for a drawing operation.

## Claims

1. A spinning process, comprising:
a. generating a plurality of molten streams from a spinneret, said streams being formed from axially extending continuous segments of dissimilar polymers arranged alternately in side-by-side temporarily adhering relationship;
b. quenching said streams to form filaments; and
c. withdrawing said filaments from said streams, said streams being selected such that first and second of said filaments have substantially the same denier and are splittable into different numbers of sub-filaments derived from said segments.

2. The process defined in claim 1, wherein said streams from which said first and said second of said filaments are quenched have substantially the same jet stretch.

3. A multi-filament yarn comprising a plurality of filaments of equal deniers splittable into sub-filaments of at least first and second polymers, at least one of said sub-filaments of said first polymer split from a first of-said filaments having a different denier than another of said sub-filaments of said first polymer split from a second of said filments.

4. The yarn defined in claim 3, wherein said first and said second of said filaments are splittable into different numbers of sub-filaments.

## Patentansprüche

1. Spinnverfahren, umfassend
a. die Erzeugung einer Vielzahl geschmolzener Ströme aus einer Spinndüse, wobei die Ströme aus sich axial erstreckenden kontinuierlichen Segmenten unterschiedlicher Polymere gebildet werden, die alternierend in einer Seite-an-Seite und zeitweilig haftenden Beziehung angeordnet sind,
b. Abschrecken der Ströme zur Bildung von Filamenten, und
c. Abziehen der Filamente von den Strömen, wobei die Ströme derart ausgewählt sind, daß das erste und zweite der Filamente im wesentlichen den selben Denierwert besitzen und in unterschiedliche Zahlen von Subfilamenten, die aus den Segmenten erhalten werden, aufspaltbar sind.

2. Verfahren nach Anspruch 1, worin die Ströme, aus denen das erste und zweite der Filamente abgeschreckt werden, in wesentlichen die selbe Düsendehnung (jet stretch) aufweisen.

3. Multifilamentgarn, enthaltend eine Vielzahl von Filamenten gleicher Denierwerte, die in Subfilamente von mindestens ersten und zweiten Polymeren aufspaltbar sind, wobei mindestens eines der Subfilamente des ersten Polymers, welches von einem ersten Filament abgespalten ist, einen anderen Denierwert aufweist als ein anderes der Subfilamente des ersten Polymers, das von einem zweiten Filament abgespalten ist.

4. Garn nach Anspruch 3, worin das erste und zweite der Filamente in eine unterschiedliche Anzahl an Subfilamenten aufspaltbar sind.

## Revendications

1. Procédé de filature, comprenant:
a. la production d'une pluralité de courants à l'état fondu à partir d'une filière, ces courants étant formés à partir de segments continus, s'étendant axialement, de polymères dissemblables disposés alternativement en relation d'adhérence temporaire côte à côte,
b. le refroidissement des courants pour former des filaments; et
c. l'extraction des filaments hors des courants, les courants étant choisis de façon que les premier et second des filaments aient sensiblement le même denier et puissent être fractionnés en nombres différents de sous-filaments obtenus à partir desdits segments.

2. Procédé selon la revendication 1, où les courants à partir desquels les premier et second des filaments sont refroidis ont sensiblement la même extension sous tuyère.

3. Filé multi-filament comprenant une pluralité de filaments de deniers égaux pouvant être fractionnés en sous-filaments d'au moins un premier et un second polymère, au moins l'un des sous-filaments du premier polymère fractionné à partir d'un premier des filaments ayant un denier différent d'un autre des sous-filaments du premier polymère fractionné à partir d'un second des filaments.

4. Filé selon la revendication 3, où le premier et le second des filaments peuvent être fractionnés en nombres différents de sous-filaments.
